

March 30, 1937.

C. E. K. MEES

2,075,048

PHOTOGRAPHIC EMULSION CONTAINING SUPERSENSITIZED CARBOCYANINES

Original Filed Nov. 4, 1932



A = A thiocarbocyanine

B = A different thiocarbocyanine

C = A combination of these two dyes

Charles E. K. Mees,

Inventor:

Daniel J. Mayne

By Walter M. Perrin

Attorneys:

Patented Mar. 30, 1937

2,075,048

# UNITED STATES PATENT OFFICE

2,075,048

## PHOTOGRAPHIC EMULSION CONTAINING SUPERSENSITIZED CARBOCYANINES

Charles E. K. Mees, Rochester, N. Y., assignor,  
by mesne assignments, to Eastman Kodak  
Company, Jersey City, N. J., a corporation of  
New Jersey

Application November 4, 1932, Serial No. 641,179  
Renewed February 9, 1935

12 Claims. (Cl. 95—7)

This invention relates to sensitized photographic emulsions and more particularly relates to photographic emulsions such as those of the gelatino-silver-halide type containing a combination of sensitizers, one of which cooperates with the other to sensitize the emulsion to a much greater degree than is possible with that sensitizer, or either sensitizer alone, or even than would be evidenced by the sum total of the sensitization produced by the two separate sensitizers individually.

In other words, I have found that the sensitivity contributed to photographic emulsions by certain sensitizers may be enhanced to a very considerable degree by adding to the basic sensitizer what I will term a "supersensitizer", the latter contributing to the emulsion the sensitivity which is peculiar to itself as well as activating or inducing further sensitivity in what I will term the "basic sensitizer". For example, a certain basic sensitizer may have a green speed of 50 H and D but when there is added thereto a supersensitizer, which may not even sensitize to the green at all (but to some other portion of the spectrum) the green speed of the basic sensitizer will be increased far beyond its original green speed. Or, assuming the basic sensitizer to sensitize the emulsion to a green speed of 50 and the supersensitizer to separately sensitize the emulsion to a green speed of 5, the addition of the supersensitizer to the basic sensitizer will sensitize the emulsion to a green speed beyond the sum total of the two separate green speeds, namely to a green speed, for instance of 80.

The combinations of sensitizers and supersensitizers which are the subject of the instant invention have the peculiar property that, in order for the supersensitizer to increase the sensitivity of the basic sensitizer, the region of sensitivity of the supersensitizer must coincide at least in part with the region of sensitivity of the basic sensitizer. The unusual effects obtained by the combinations of sensitizers which constitute the instant invention result, therefore, from the unusual influence or relation which the supersensitizers have upon or to the respective basic sensitizers.

Accordingly, it is among the objects of my invention to provide a photographic emulsion which contains a basic sensitizer for the emulsion and which also contains a supersensitizer which contributes its own individual sensitization to the emulsion and also increases the sensitization caused by the basic sensitizer. It is a further object of my invention to provide certain combinations or mixtures of sensitizers in a photographic emulsion which will contribute to the emulsion a sensitivity (ability to respond to light) not heretofore obtainable with either of the individual sensitizers in the combination.

Other objects will become apparent to those skilled in the art upon a further perusal of this specification.

I have found, for instance, that the sensitivity which the thiocarbocyanines contribute to a gelatino-silver-halide emulsion will be markedly increased if there is present in the photographic emulsion along with each part of the thiocarbocyanine, from approximately  $\frac{1}{10}$  part or even less to approximately one part or even more of a 2:2' dialkyl 8 alkyl dibenzothiocarbocyanine salt as a supersensitizer. I find this supersensitizing effect upon the sensitizing properties of the thiocarbocyanines to be general with or representative of the 2:2' dialkyl 8 alkyl dibenzothiocarbocyanine salts which themselves have the ability of separately sensitizing photographic emulsions. The best results are obtained, however, where the thiocarbocyanine used as the basic sensitizer is substituted in the central position of the trimethenyl chain by an alkyl group.

Referring to the attached drawing, forming a part hereof, there is represented a hypothetical wedge spectrogram illustrating my invention. The curve A shows the approximate sensitivity conferred upon a gelatino-silver-halide emulsion by a 2:2' dialkyl 8 alkyl thiocarbocyanine salt as a basic sensitizer. The curve B illustrates diagrammatically the sensitivity separately conferred upon the same gelatino-silver-halide emulsion by a 2:2' dialkyl 8 alkyl dibenzothiocarbocyanine salt. The curve C, however, illustrates the sensitivity of the same photographic emulsion containing a small percentage of a solution in which is dissolved approximately equal parts of these two salts. From this it will be apparent that the combination or mixture of these sensitizers contributes to the photographic emulsion a sensitivity far beyond that which it is possible to obtain even from the sum total of the sensitization resulting from the individual sensitizers.

More specifically my invention is accomplished by dissolving the sensitizing dyes in, for instance, methyl alcohol. The sensitizer and supersensitizer are added to the alcohol, for instance, in equal proportions, although I have found that less than an equal amount of the supersensitizer is normally sufficient to confer upon the sensitizer an increased sensitivity. For example, while I may dissolve in the methyl alcohol solvent one part of the 2:2' dialkyl 8 alkyl thiocarbocyanine salt, I may then add to the alcohol from  $\frac{1}{10}$  part or even less to one part or even more of the 2:2' dialkyl 8 alkyl dibenzothiocarbocyanine salt, depending upon the effect that is desired in the photographic emulsion. The exact ratio of the supersensitizer to the sensitizer is not particularly important inasmuch as those skilled in the art can readily determine by what ratio the greatest degree of sensitization of the basic sensitizer can be obtained.

This solution of the sensitizer and supersensitizer is then diluted with water and a volume containing from a few milligrams to as much as 100 milligrams, and preferably from about 10 to 30 milligrams of the sensitizers, is then added to 5 1000 cc. of a gelatino-silver-halide emulsion, such as is customarily employed in the art. Obviously, if the basic sensitizer is greatly supersensitized by the supersensitizer, less of the sensitizer combination will be necessary to obtain the desired 10 degree of sensitization in the emulsion. The emulsion may then be coated upon a transparent support as is well known in the art, either glass, or a cellulose nitrate or acetate, or other cellulose 15 derivative, base being satisfactory as the support.

As further illustrating my invention, I have tabulated hereinafter typical examples of dibenzothiocarbocyanines which themselves have 20 the power of sensitizing a photographic emulsion and also have the ability of supersensitizing the sensitizing effect of the carbocyanines on the photographic emulsion. Compounds which are characteristic of those which I may employ as 25 supersensitizers for the carbocyanines opposite which they are set, are as follows—

| Basic sensitizer                                                | Supersensitizer                                                 |
|-----------------------------------------------------------------|-----------------------------------------------------------------|
| 30 2:2' dimethyl 8 ethyl thiocarbocyanine iodide.               | 2:2' diethyl 8 methyl 3:4:3':4' dibenzothiocarbocyanine iodide. |
| 2:2' diethyl 8 methyl thiocarbocyanine iodide.                  |                                                                 |
| 4 phenyl neo thiazolo carbocyanine iodide.                      |                                                                 |
| 2:2' dimethyl 8 ethyl 3:4:3':4' dibenzothiocarbocyanine iodide. | 2:2' dimethyl 8 ethyl 3:4:3':4' dibenzothiocarbocyanine iodide. |
| 35 2:2' dimethyl 8 methyl thiocarbocyanine iodide.              | 2:2' dimethyl 8 ethyl 3:4:3':4' dibenzothiocarbocyanine iodide. |
| 2:2' diethyl 8 methyl thiocarbocyanine iodide.                  |                                                                 |
| 2:2' dimethyl 5:5':8 triethyl thiocarbocyanine iodide.          |                                                                 |
| 2:2':5:8 pentaethyl thiocarbocyanine iodide.                    |                                                                 |
| 40 2:2' dimethyl 8 ethyl thiocarbocyanine iodide.               |                                                                 |

Other examples showing the broad application of my invention could be cited, although the foregoing will be sufficient to teach those skilled in the art the manner in which my invention is carried out and the broad principle of supersensitizing basic sensitizers of numerous types with compounds which themselves have separate sensitizing properties and the regions of spectral sensitivity 45 of which coincide at least in part with the respective spectrograms of the basic sensitizers. For instance, the thiocarbocyanines and the dibenzothiocarbocyanines, unsubstituted in the 8-position, respond to supersensitization by the 50 supersensitizers herein in the same manner but not to the same degree as do the 8-substituted thiocarbocyanines. The selenium containing carbocyanines may also be used as basic sensitizers in the same manner as the thiocarbocyanines described herein, although they do not respond to 55 supersensitization to the same degree. I have also found that the 2:2' dimethyl 8 ethyl 3:4:3':4' dibenzothiocarbocyanine is very markedly supersensitized by both 2:2' diethyl 8 methyl 3:4:3':4' 60 dibenzothiocarbocyanine iodide and 2:2' dimethyl 8 ethyl 3:4:3':4' dibenzothiocarbocyanine iodide, following the procedure outlined above.

Numerous variations to the above invention 65 will doubtless occur to those skilled in the art and will be included in the scope of my invention as defined by the claims appended hereto, it being understood that the foregoing is merely illustrative of the manner of practicing my invention and the results to be obtained thereby.

What I claim as my invention and desire to be secured by Letters Patent in the United States is:

1. A gelatino-silver-halide emulsion containing two sensitizers for the emulsion, one of which is a carbocyanine selected from the group consisting of thiocarbocyanines and selenocarbocyanines, as a basic sensitizer, and the other of which is a dibenzothiocarbocyanine, as a supersensitizer.

2. A gelatino-silver-halide emulsion containing two sensitizers for the emulsion, one of which is a thiocarbocyanine, as a basic sensitizer, and the other of which is a dibenzothiocarbocyanine, as a supersensitizer.

3. A gelatino-silver-halide emulsion containing two sensitizers for the emulsion, one of which is a selenocarbocyanine, as a basic sensitizer, and the other of which is a dibenzothiocarbocyanine, as a supersensitizer.

4. A gelatino-silver-halide emulsion containing two sensitizers for the emulsion, one of which is a thiocarbocyanine substituted at the central carbon atom of the trimethenyl chain, as a basic sensitizer, and the other of which is a dibenzothiocarbocyanine, as a super-sensitizer.

5. A gelatino-silver-halide emulsion containing two sensitizers for the emulsion, one of which is 2:2' dialkyl 8 alkyl thiocarbocyanine halide, as a basic sensitizer, and the other of which is 2:2' dialkyl 8 alkyl dibenzothiocarbocyanine halide, as a supersensitizer.

6. A gelatino-silver-halide emulsion containing two different sensitizers for the emulsion, one of which is 2:2' dialkyl 8 alkyl dibenzothiocarbocyanine halide, as a basic sensitizer, and the other of which is 2:2' dialkyl 8 alkyl dibenzothiocarbocyanine halide, as a supersensitizer.

7. A gelatino-silver-halide emulsion containing two sensitizers for the emulsion, one of which is 2:2' dimethyl 8 ethyl thiocarbocyanine iodide, as a basic sensitizer, and the other of which is 2:2' diethyl 8 methyl 3:4:3':4' dibenzothiocarbocyanine iodide, as a supersensitizer.

8. A gelatino-silver-halide emulsion containing two sensitizers for the emulsion, one of which is 2:2' diethyl 8 methyl thiocarbocyanine iodide, as a basic sensitizer, and the other of which is 2:2' diethyl 8 methyl 3:4:3':4' dibenzothiocarbocyanine iodide, as a supersensitizer.

9. A gelatino-silver-halide emulsion containing two sensitizers for the emulsion, one of which is 2:2' diethyl 8 methyl thiocarbocyanine iodide, as a basic sensitizer, and the other of which is 2:2' dimethyl 8 ethyl 3:4:3':4' dibenzothiocarbocyanine iodide, as a supersensitizer.

10. A gelatino-silver-halide emulsion containing two sensitizers for the emulsion, one of which is 2:2' dimethyl 8 ethyl thiocarbocyanine iodide as a basic sensitizer, and the other of which is 2:2' dimethyl 8 ethyl 3:4:3':4' dibenzothiocarbocyanine iodide, as a supersensitizer.

11. A photographic element comprising a gelatino-silver-halide emulsion containing two sensitizers for the emulsion, one of which is a thiocarbocyanine, as a basic sensitizer, and the other of which is a dibenzothiocarbocyanine, as a supersensitizer.

12. A photographic element comprising a gelatino-silver-halide emulsion containing two sensitizers for the emulsion, one of which is a selenocarbocyanine, as a basic sensitizer, and the other of which is a dibenzothiocarbocyanine, as a supersensitizer.

CHARLES E. K. MEES.